

[54] PHOTOCOCONDUCTIVE POLYMERS OF THIOCYANO-SUBSTITUTED-9-VINYLCARBAZOLES

[75] Inventors: **Takeshi Fida**, Chiba; **Katsuhiko Nishide**, Tokyo; **Teruo Yamanouchi**, Fujisawa; **Kikuo Kinjo**, Tokyo, all of Japan

[73] Assignee: **Canon Kabushiki Kaisha**, Tokyo, Japan

[22] Filed: **July 18, 1974**

[21] Appl. No.: **489,530**

**Related U.S. Application Data**

[63] Continuation of Ser. No. 396,700, Sept. 13, 1973, abandoned, which is a continuation of Ser. No. 195,852, Nov. 4, 1971, abandoned.

[30] **Foreign Application Priority Data**

Nov. 9, 1970 Japan..... 45-98528

[52] **U.S. Cl.**..... **96/1.5; 260/79.5 R; 260/79.7; 260/88.3 R; 96/1.6**

[51] **Int. Cl.<sup>2</sup>** ..... **G03G 5/06**

[58] **Field of Search**..... 96/1.5, 1.6; 260/79.5 R, 260/79.7, 315, 88.3 R

[56] **References Cited**

UNITED STATES PATENTS

|           |         |                  |          |
|-----------|---------|------------------|----------|
| 3,287,121 | 11/1966 | Hoegl.....       | 96/1.5   |
| 3,418,116 | 12/1968 | Inami et al..... | 96/1.5   |
| 3,421,891 | 1/1969  | Inami et al..... | 96/1.6   |
| 3,542,546 | 11/1970 | Fox.....         | 96/1.5   |
| 3,627,524 | 12/1971 | Kinjo et al..... | 96/1.6 X |

FOREIGN PATENTS OR APPLICATIONS

|           |        |            |        |
|-----------|--------|------------|--------|
| 4,114,508 | 8/1966 | Japan..... | 96/1.5 |
| 437,592   | 3/1968 | Japan..... | 96/1.5 |

*Primary Examiner*—Roland E. Martin, Jr.  
*Attorney, Agent, or Firm*—Fitzpatrick, Cella, Harper & Scinto

[57]

**ABSTRACT**

An electrophotographic photosensitive materials comprises a polymer containing a moiety of cyano or thiocyanato substituted 9-vinylcarbazole unit.

4 Claims, No Drawings

PHOTOCONDUCTIVE POLYMERS OF  
THIOCYANO-SUBSTITUTED-9-VINYLCAR-  
BOZOLES

This is a continuation of application Ser. No. 396,700, filed Sept. 13, 1973, now abandoned, which is a continuation of Ser. No. 195,852, filed Nov. 4, 1971, now abandoned.

BACKGROUND OF THE INVENTION

1. Field of the Invention

This invention relates to an electrophotographic photosensitive material.

2. Description of the Prior Art

There have been known various organic photoconductive materials for electrophotographic photosensitive members. However, conventional organic photoconductive materials are of low sensitivity, and the sensitivity has not been improved without deteriorating the color tone of the photosensitive layer, glassy uniformity and flexibility.

Organic photoconductors of high polymer type have been also known. For example, there may be mentioned polymers having heterocyclic moiety such as carbazole ring and polymers containing polynuclear aromatic ring moiety such as naphthalene ring, anthracene ring and the like.

These organic high polymer conductors have various advantages such as transparency, light weight and film-shapeability and are expected to be used widely. Nevertheless they are not practically used since their photo-sensitivity is disadvantageously far lower and the physical property is not better than conventional inorganic photoconductors.

SUMMARY OF THE INVENTION

According to this invention, the electrophotographic photosensitive materials comprises a polymer containing a moiety of cyano or thiocyan substituted 9-vinylcarbazole unit having the formula:



where R is a member selected from the group consisting of hydrogen, chloro, bromo, iodo and nitro.

An object of this invention is to provide an electrophotographic photosensitive material of high sensitivity and low remaining potential when exposed.

Another object of this invention is to provide an electrophotographic photosensitive material having good physical properties.

DESCRIPTION OF THE PREFERRED  
EMBODIMENTS

Representative polymers having cyano substituted 9-vinylcarbazole recurring moiety are cyano substituted poly-9-vinylcarbazole, cyano substituted copolymers of 9-vinylcarbazole with acrylic acid ester, methacrylic acid ester or styrene, and cyano substituted halogenated poly-9-vinylcarbazole.

Representative polymers having thiocyanato substituted 9-vinylcarbazole recurring moiety are thiocyanato

substituted poly-9-vinylcarbazole, thiocyanato substituted copolymer of 9-vinylcarbazole with acrylic acid ester, methacrylic acid ester, or styrene, thiocyanato substituted halogenated 9-vinylcarbazole homopolymers or copolymers.

The copolymers are prepared for the purpose of improving film-shapeability, flexibility and solubility by introducing a monomer unit suitable therefore.

When the monomer unit does not have photoconductivity, sensitivity of the resulting copolymer is generally lowered, but this lowering is compensated by cyanogenation or thiocyanation.

The mechanism by which the electrophotographic photosensitive material of the instant invention shows high sensitivity and high photoconductivity is not clear, but it is considered that the 9-vinylcarbazole ring moiety behaves as donor and cyano and thiocyanato groups behave as acceptor and there occurs intramolecular charge transfer.

When the polymer of the instant invention is a copolymer containing cyano- or thiocyanato substituted 9-vinylcarbazole unit, the copolymer may contain the following monomer units in addition to those as mentioned previously: 2-vinylpyridine, vinylanthracene,

vinylnaphthalene, styrene, acrylonitrile, methyl acrylate, ethyl acrylate, vinyl acetate, vinylidene chloride, vinyl carbazole, halogen-, nitro- or amino-substituted vinylcarbazole, vinyl stearate, n-butyl acrylate, acyloxyethylidethylamine, vinyl cinnamate, ethylene, vinyl pyrrolidone, vinyl chloride and the like.

The copolymers of the present invention may contain two or more monomer units in addition to the cyano- or thiocyanato-substituted vinylcarbazole monomer unit.

The polymers containing cyano- or thiocyanato vinylcarbazole unit of the instant invention may be prepared by various organic synthesis methods. Representative examples thereof are shown below.

1. 9-Vinylcarbazole having a halogen substituent or derivative thereof is homopolymerized or copolymerized and then reacted with a cyanide.

2. Homopolymer or copolymer of 9-vinylcarbazole or derivative thereof is halogenated by a conventional method and then reacted with a cyanide.

It has been found that in the reactions (1) or (2) above the halogen atom particularly bromine and iodine atom present at 3- or 6-position of the carbazole nucleus is smoothly replaced by a cyano group when the carbazole ring is treated by heating with cuprous cyanide in a non-proton polar solvent such as dimethylformamide, dimethylacetamide, N-methylpyrrolidone and the like. The resulting percentage of replacement of halogen atom depends on kind of halogen and reaction conditions, but at an optimum condition it amounts to almost 100%.

In the above reaction, gellation hardly occurs during the reaction procedure and after the end product has been obtained.

Examples of homopolymer or copolymer of 9-vinylcarbazole or derivative thereof to which cyano or thiocyanato group is to be introduced are shown below.

A. Homopolymers of 9-vinylcarbazole having a halogen substituent:

homopolymer derived from monomers such as

3-bromo-9-vinylcarbazole,

3-iodo-9-vinylcarbazole,

3-chloro-6-bromo-9-vinylcarbazole,

3, 6-diiodo-9-vinylcarbazole,

3-chloro-9-vinylcarbazole,

3, 6-dichloro-9-vinylcarbazole,  
 3-chloro-6-iodo-9-vinylcarbazole and the like.  
**B. Copolymer of 9-vinylcarbazole having a halogen substituent:**  
 copolymer of a monomer described (A) above with a monomer such as  
 2-vinylpyridine,  
 vinylanthracene,  
 vinylnaphthalene,  
 styrene,  
 acrylonitrile,  
 methyl acrylate,  
 ethyl acrylate,  
 vinyl acetate,  
 vinylidene chloride,  
 vinylcarbazole,  
 nitro substituted vinylcarbazole,  
 amino substituted vinylcarbazole,  
 halogen substituted vinylcarbazole (excluding combinations with the same one as mentioned in A) above),  
 vinyl stearate,  
 n-butyl acrylate,  
 acryloxydiethylamine,  
 vinylcinnamate,  
 ethylene,  
 vinylpyrrolidone,  
 vinylchloride, and the like.

**C. Homopolymers of 9-vinylcarbazole derivative having a halogen substituent:**

homopolymer derived from monomers such as  
 3-bromo-6-nitro-9-vinylcarbazole,  
 3-chloro-6-nitro-9-vinylcarbazole.

**D. Copolymers of monomers described in (C) above with monomers described in (B) above (as copolymer of 9-vinylcarbazole derivative).** 3. Cyano group may be introduced into homopolymer or copolymers of 9-vinylcarbazole or 9-vinylcarbazole derivative by Friedel-Crafts reaction with cyanogen bromide.

Preparation examples of cyano substituted poly-9-vinylcarbazoles are shown below.

#### PREPARATION EXAMPLE 1

5.0 g. of poly-9-vinylcarbazole was dissolved in 50 cc. of pyridine and 6.6 g. of iodine was added thereto and stirred for 3 hours at 110° C. After cooled, the solution was poured into a large amount of methanol to precipitate the resulting polymer. The polymer was filtered, dried and purified by reprecipitating in pyridine-methanol. The polymer thus obtained was an iodinated poly-9-vinylcarbazole and contained 20.49 % of iodine according to elementary analysis.

2.0 g. of the iodinated poly-9-vinylcarbazole was dissolved in 50 cc of N-methyl-2-pyrrolidone, and 0.5 g. of cuprous cyanide was added thereto and stirred at 150° C for 6 hours. After cooled, the above mixture was poured into a large amount of methanol to precipitate the polymer thus produced and the polymer thus pre-

5  
 10  
 15  
 20  
 25  
 30  
 35  
 40  
 45  
 50

cipitated was filtered, dried and purified by reprecipitating in pyridine-methanol to give white polymer. This white polymer is soluble in organic solvents such as tetrahydrofuran, pyridine, chlorobenzene and the like. Infrared absorption spectrum of the polymer shows absorptions at 2210  $\text{cm}^{-1}$  for cyano, and 890  $\text{cm}^{-1}$  and 805  $\text{cm}^{-1}$  for 3-position substituent of carbazole ring. Elementary analysis shows that there is contained 9.65 % of nitrogen, but not any iodine. This result consists with the calculated values.

Consequently this reaction is quantitative and the resulting polymer is mainly cyano substituted poly-9-vinylcarbazole having cyano substituent at 3-position of carbazole ring which contains average 0.39 cyano groups per carbazole ring.

#### PREPARATION EXAMPLE 2

Following Preparation Example 1, there were prepared many iodinated poly-9-vinylcarbazoles having a cyano substituent.

By adjusting the preparation conditions, cyano substituting degree can be controlled. General relations between preparation conditions and cyano substituting degree, are as shown below.

Degree of substitution of iodine in poly-9-vinylcarbazole can be controlled to less than 1.35 atom per vinylcarbazole ring (hereinafter, degree of substitution is designated as "per vinylcarbazole ring"). In the present Preparation Example, the starting material is a poly-9-vinylcarbazole having degree of iodine substitution of 0.183 to 0.706 atom. The conversion degree of iodine to cyano can amount to 90 to 95 % depending upon selection of preparation conditions. Solvents used in preparation of iodinated poly-9-vinylcarbazole are preferably pyridine (capable of dissolving a cyano substituted polymer having up to about 0.7 cyano group per carbazole ring), tetrahydrofuran (capable of dissolving a cyano substituted polymer having up to about 0.6 cyano group per carbazole ring) and monochlorobenzene (capable of dissolving a cyano substituted polymer having up to about 0.4 cyano group per carbazole ring).

As reaction solvent, N-methylpyrrolidone is most preferable but pyridine is also preferable. The reaction temperature is 150° C when N-methylpyrrolidone is used. There is obtained white polymer easily soluble in solvent. Conversion degree of cyano group is 20 to 95% and the sample is obtained by a reaction for 6-8 hours. The conversion degree amounts to as high as 100 % at 200° C for 2 hours, but there are formed colored polymer of low solubility. The amount of cuprous cyanide is preferably about up to 2 moles per 1 mole of iodine. Amount of cuprous cyanide higher than that hardly contributes to substitution degree of cyano group. The preparation conditions and elementary analysis in the present preparation examples are shown in the table below, where "%" is percent by weight.

| No.   | Analysis:<br>iodine % | Iodine content<br>in iodinated<br>PVCZ *1 | CuCN/1<br>molar<br>ratio | Reaction<br>time<br>(hr.) | CN content<br>*2 | PVCZ<br>I content<br>*3 | chloro-<br>benzene | Solubility<br>tetra-<br>hydrofuran | Py-<br>ridine | Color |
|-------|-----------------------|-------------------------------------------|--------------------------|---------------------------|------------------|-------------------------|--------------------|------------------------------------|---------------|-------|
| 1 - 1 | 2.67                  | 0.183                                     | 2                        | 6                         | 0.140            | 0.043                   | 0                  | 0                                  | 0             | White |
| 1 - 2 | 3.43                  | 0.287                                     | 2                        | 4                         | 0.231            | 0.056                   | 0                  | 0                                  | 0             | White |
| 1 - 3 | 1.82                  | 0.327                                     | 2                        | 6                         | 0.298            | 0.009                   | 0                  | 0                                  | 0             | White |
| 1 - 4 | 11.84                 | 0.392                                     | 2                        | 2                         | 0.183            | 0.109                   | 0                  | 0                                  | 0             | White |
| 1 - 5 | 4.94                  | 0.405                                     | 2                        | 4                         | 0.323            | 0.082                   | X                  | 0                                  | 0             | White |
| 1 - 6 | 3.91                  | 0.405                                     | 5                        | 4                         | 0.339            | 0.066                   | 0                  | 0                                  | 0             | White |

-continued

| No.    | Analysis:<br>iodine % | Iodine content<br>in iodinated<br>PVCZ: <sup>*1</sup> | CuCN/1<br>molar<br>ratio | Reaction<br>time<br>(hr.) | Cyanate<br>CN content<br><sup>*2</sup> | PVCZ<br>I content<br><sup>*3</sup> | chloro-<br>benzene | Solubility<br>tetra-<br>hydrofuran | Py-<br>ridine | Color |
|--------|-----------------------|-------------------------------------------------------|--------------------------|---------------------------|----------------------------------------|------------------------------------|--------------------|------------------------------------|---------------|-------|
| 1 - 7  | 5.10                  | 0.416                                                 | 2                        | 3                         | 0.331                                  | 0.085                              |                    | 0                                  | 0             | White |
| 1 - 8  | 1.97                  | 0.416                                                 | 2                        | 8                         | 0.384                                  | 0.032                              | X                  | 0                                  | 0             | White |
| 1 - 9  | 2.18                  | 0.610                                                 | 2                        | 6                         | 0.374                                  | 0.036                              | X                  | 0                                  | 0             | White |
| 1 - 10 | 1.78                  | 0.610                                                 | 2                        | 8                         | 0.580                                  | 0.030                              | X                  | 0                                  | 0             | White |

The reaction was effected in a solvent of N-methyl-2-pyrrolidone at 150°C.

0 : highly soluble  
1 : soluble

X : low solubility

PVCZ : poly-9-vinylcarbazole

\*1 Iodine atom/carbazole ring

\*2 CN group/carbazole ring

\*3 Iodine atom/carbazole ring

### PREPARATION EXAMPLE 3

5.0 g. of brominated poly-9-vinylcarbazole (bromine content, 43.28 %; produced by brominating poly-9-vinylcarbazole by Wohl-Ziegler reaction or brominating poly-9-vinylcarbazole with bromine in pyridine) was dissolved in 50 cc. of pyridine, and 0.8 g. of cuprous cyanide was added thereto and reacted at 110°C for 8 hours. After cooled, the reaction solution was poured into a large amount of methanol to precipitate the resulting polymer, which was then filtered, dried, and purified by reprecipitating the polymer in pyridine-methanol to obtain white polymer. Infrared absorption spectrum shows remarkable characteristic absorption at 2210  $\text{cm}^{-1}$ , 890  $\text{cm}^{-1}$  and 805  $\text{cm}^{-1}$  as in Preparation Example 1 and bromine content is 24.70 % as the result of elementary analysis. Therefore, it is found that the polymer product is cyano substituted brominated poly-9-vinylcarbazole having average 0.94 cyano group and average 0.89 bromine mainly at 3-position and 6-position of carbazole ring.

Reaction of brominated poly-9-vinylcarbazole with cuprous cyanide takes longer time than that of iodinated poly-9-vinylcarbazole with cuprous cyanide. Conversion degree of bromo substituent to cyano is lower than that of iodo substituent to cyano. The other example is shown below.

poly-9-vinylcarbazole of chlorine content of 4.69 % obtained by chlorinating poly-9-vinylcarbazole with sulfonyl chloride was treated with 8.4 f. of iodine in a way similar to Preparation Example 1). Cuprous cyanide (1.2 g.) was added thereto and reacted at 110°C for 10 hours. The resulting product was treated in a way similar to Preparation Example 1 and there was obtained white cyano substituted chlorinated poly-9-vinylcarbazole (elementary analysis, found: halogen, 4.61 %; N, 8.48). This elementary analysis is consistent with calculated values of halogen and nitrogen in case where all iodine are replaced by cyano group.

This result of elementary analysis indicates that average degrees of cyano and chlorine per carbazole ring were 0.25 and 0.27, respectively.

### PREPARATION EXAMPLE 5

5.0 g of iodinated poly-9-vinylcarbazole (iodine content, 20.49 %) shown in Preparation Example 1 was dissolved in 125 cc. of N-methyl-2-pyrrolidone, and 0.80 g. of cuprous cyanide was added thereto and stirred at 150°C for 8 hours followed by treating in a way similar to Preparation Example 1 to produce white polymer soluble in organic solvents. The infrared absorption spectrum shows characteristic absorption at 2210  $\text{cm}^{-1}$  for cyano and characteristic absorptions at 890 and 805  $\text{cm}^{-1}$  for 3-position substituent in carbazole ring. Elementary analysis shows 6.80 % of iodine content. These data indicate that the resulting polymer is mainly cyano substituted iodinated poly-9-vinylcarbazole having average 0.28 cyano groups and 0.12 iodine at 3-position.

Preparation of polymers containing cyano substituted 9-vinylcarbazole moiety may be carried out by cyanogenation of 9-vinylcarbazole or 9-vinylcarbazole derivative and then polymerizing the cyanogenated

| Br content in<br>brominated poly-9-<br>vinylcarbazole<br>(atom/carbazole ring) | Brominated poly-9-<br>vinylcarbazole<br>g. | Feed<br>N-methyl<br>pyrrolidone<br>ml.  | CuCN<br>g.                             | CuCN/Br<br>molar<br>ratio         |
|--------------------------------------------------------------------------------|--------------------------------------------|-----------------------------------------|----------------------------------------|-----------------------------------|
| 0.706                                                                          | 5                                          | 125                                     | 2.67                                   | 4                                 |
| Reaction condition                                                             |                                            |                                         |                                        |                                   |
| Reaction<br>temperature<br>°C                                                  | Reaction<br>Time<br>hr.                    | Cyano substituted poly-9-vinylcarbazole |                                        |                                   |
| 150                                                                            | 40                                         | CN content<br>(atom/carbazole<br>ring)  | Br content<br>(atom/carbazole<br>ring) |                                   |
|                                                                                |                                            | 0.223                                   | 0.483                                  |                                   |
|                                                                                |                                            | Solubility                              |                                        |                                   |
|                                                                                |                                            | Pyridine<br>easily<br>soluble           | THF<br>easily<br>soluble               | Monochloro-<br>benzene<br>soluble |
|                                                                                |                                            |                                         |                                        | Color<br>slightly<br>brown        |

### PREPARATION EXAMPLE 4

In 50 cc. of pyridine was added 5.0 g. of chlorinated iodinated poly-9-vinylcarbazole (chlorine content, 4.07 %; iodine content, 13.33 %; 10 g. of chlorinated

one.

65

### PREPARATION EXAMPLE 6

3.2 g. of 3-iodo-9-vinylcarbazole (m.p. 194°C. dec., produced by iodination of 9- $\beta$ -chloroethylcarbazole

and dehydration with potassium hydroxide) was dissolved in 50 cc. of N-methyl-2-pyrrolidone, and 2.0 g. of Cu CN was added thereto and a small amount of hydroquinone was added and heated in an atmosphere of nitrogen at 150° C with stirring. The reaction mixture was poured into water, filtered, washed with water, dried and recrystallized three times to give 1.5 g. of 3-cyano-9-vinylcarbazole.

Analysis: Found N, 11.5 %. Calcd. N, 12.9 %.

0.5 g. of the resulting 3-cyano-9-vinylcarbazole and 1.0 g. of 9-vinylcarbazole were placed in a polymerization tube and azobisisobutyronitrile was added and heated at 80°C for 8 hours in nitrogen atmosphere. The polymer was dissolved in tetrahydrofuran and precipitated in methanol. White polymer easily soluble in tetrahydrofuran was obtained. The resulting polymer contains about 31 % of 3-cyano-9-vinylcarbazole.

Thiocyanated polymer may be prepared, for example, as follows.

1. A process for making a substitution of thiocyanato group to poly-9-vinylcarbazole or copolymer of 9-vinylcarbazole;

2. A process for thiocyanating halogenated 9-vinylcarbazole homopolymer or copolymer; and

3. A process for halogenating homopolymer or copolymer of thiocyanated 9-vinylcarbazole.

The thiocyanation reaction may be carried out by methods described in "Organic Reactions", Vol. 3, page 240 and the following pages (edited by R. Adams) or modified method thereof. There may be mentioned

a. a process for adding a solution of free thiocyanogen in benzene, chlorobenzene, chloroform or methylene chloride to a solution of 9-vinylcarbazole polymer; and

b. a process for making a reaction by forming thiocyanogen electrobatically or chemically (e.g. alkali metal thiocyanate and halogen). Some poly-9-vinylcarbazoles highly substituted with thiocyanato group are insoluble in benzene and monochlorobenzene and in this case it is advantageous to effect the reaction in tetrahydrofuran and dioxane. Further, the above-mentioned homopolymer or copolymer in (A)-(D) may be thiocyanated. Thiocyanated 9-vinylcarbazole or 9-vinylcarbazole derivative may be polymerized.

In the following there are described preparation Examples of thiocyanated 9-vinylcarbazole homopolymer and copolymer.

#### PREPARATION EXAMPLE 7

Poly-9-vinylcarbazole (3.9 g.) was dissolved in 180 ml. of monochlorobenzene, and a solution of thiocyanogen (obtained from lead thiocyanate and equivalent bromine) in monochlorobenzene was added thereto with stirring at -5° to -10°C and reacted for 3 hours.

The reaction mixture was poured into methanol to precipitate the resulting polymer and the polymer was further washed with methanol and dried under reduced pressure.

55

60

65

| Polymer | Amount of thiocyanogen | Reaction temperature | Yield   |
|---------|------------------------|----------------------|---------|
| " (1)   | 0.58 g.                | 20°C                 | 4.1 gr. |
| " (2)   | 1.16 g.                | 20°C                 | 4.4 gr. |

Elementary analysis of the resulting polymer is shown below.

|    |             | N      | S      |                                     |
|----|-------------|--------|--------|-------------------------------------|
| 5  | Polymer (1) | 8.24 % | 3.85 % | easily soluble in monochlorobenzene |
| 10 | " (2)       | 9.50   | 7.18   | "                                   |

In infrared absorption spectrum there appear 2145  $\text{cm}^{-1}$  ( $-\text{C}=\text{N}$ ), 860  $\text{cm}^{-1}$  and 790  $\text{cm}^{-1}$  (1, 3, 4-substituted benzene nucleus) and these wave numbers indicate that SCN group mainly attaches to 3-position of the carbazole ring.

#### PREPARATION EXAMPLE 8

Cupric thiocyanate 2.0 g. (obtained by adding potassium thiocyanate to an aqueous solution of cupric sulfate, filtering the resulting precipitate and washed with ethanol and then ether) was suspended in a solution of 3.9 g of poly-9-vinylcarbazole in 180 ml. of monochlorobenzene and 25 ml. of glacial acetic acid and stirred at 30°-50°C. After the black cupric thiocyanate becomes almost white, the reaction liquid is subjected to centrifugal treatment to remove insoluble matters and then poured into methanol to precipitate polymer, filtered, washed with methanol and dried under reduced pressure. Analysis of the resulting polymer: Found: N, 9.50; S, 7.02 %.

#### PREPARATION EXAMPLE 9

10 g. of 9-vinylcarbazole-ethyl acrylate copolymer (9-vinylcarbazole, 71 mole %) was dissolved in 200 ml. of monochlorobenzene and 20 ml. of pyridine and 40 ml. of benzene containing 2.5 g. of thiocyanogen was added dropwise at 10°C with stirring. After completion of the addition, the reaction was carried out further for 2 hours at the same temperature and the reaction liquid was poured into a large amount of methanol to precipitate the copolymer. The copolymer was washed with methanol and dried under vacuum.

Analysis: Found: N, 7.92%; S, 6.05 %.

Following the above preparation procedure except for using 9-vinylcarbazole-styrene copolymer (9-vinylcarbazole, 95 mole %) in place of 9-vinylcarbazole-ethyl acrylate copolymer, there was obtained thiocyanated 9-vinylcarbazole-styrene copolymer.

Analysis: N, 9.30%; S, 7.41 %.

#### PREPARATION EXAMPLE 10

4 g. of poly-9-vinylcarbazole was dissolved in 200 ml. of dry methylene chloride, and 5 ml. of methylene chloride containing 1.4 g. of sulfonyl chloride was added dropwise at 0°C. Then, the reaction was effected for 3 hours at 20° C and the reaction mixture was poured into a large amount of methanol and the polymer thus precipitated was filtered and dried. Yield 4.3 g.

Analysis: Cl, 8.38%; N, 6.40 %.

The chlorinated poly-9-vinylcarbazole (21 g.) thus obtained was dissolved in 50 ml. of monochlorobenzene and 5ml. of benzene containing 0.6 g. of thiocyanogen was added dropwise with stirring at 10°C.

After completion of addition, the stirring was continued for further 2 hours at the same temperature and the reaction mixture was poured into a large amount of methanol.

The polymer product thus precipitated was collected and purified by recrystallizing in monochlorobenzene-methanol. Analysis: N, 8.64%; Cl, 7.39%; S, 6.72%.

The polymers as obtained above may be made into electrophotographic photosensitive member, for example, by coating a solution of the polymer on a conductive support followed by drying, or melt-coating the polymer on a conductive support, or forming a self-supporting polymer film by melt-extruding or evaporating a solvent from the polymer solution.

The polymer may be used as electrophotographic photosensitive member in a form of self-supporting film or textile or a thin film on a conductive support. For example, the polymer solution is coated on a glass plate, dried and then film is peeled off and the polymer melt is extruded through a nozzle to form fiber and then woven, or the polymer solution was coated on a conductive support.

To the polymer there may be added additives for adjusting photographic characteristics such as sensitizer and additives for adjusting physical properties such as plasticizer and opaque-rendering agent.

As sensitizers, there may be mentioned, for example, Lewis acid sensitizers, polynitro compounds such as 1, 3, 5-trinitrobenzene, picric acid, 5-nitroacenaphthene and 2, 4, 7-trinitrofluorenone; carboxylic acid such as acetic acid, trifluoroacetic acid, trichloroacetic acid, and salicylic acid; sulfonic acid such as benzene sulfonic acid and p-toluene sulfonic acid; sulfonic acid chloride such as p-toluene sulfonic acid chloride; and optical sensitizers such as Crystal Violet, Malachite Green, Methylene Blue, Brilliant Green, and Quinizarin.

As plasticizers, there may be mentioned dibutyl phthalate, dioctyl phthalate, tricresyl phosphate and chlorinated polyphenyl.

Organic photoconductive are usually used together with a dye sensitizer or Lewis acid sensitizer since even the highest sensitive organic photoconductive materials are still fairly less sensitive than inorganic photoconductive materials.

The organic photoconductive materials of this invention are also excellent in light decay characteristics and photosensitivity, and it is preferable to use practically them together with various dye sensitizers and Lewis acid.

One of the most effective sensitization method for the organic photoconductive material of the present invention is free radical sensitization. Free radical sensitization may be carried out as shown below. To the organic photoconductive material of the present invention is added a free radical former in an amount of about 1-30% by weight on the basis of the organic photoconductive polymer and radiation such as ultraviolet ray or color light is applied thereto for from several minutes to several tens minutes, and the resulting sensitivity is comparable to color-sensitized zinc oxide.

Representative examples of free radical former are polyhalogen compounds such as  $\text{CBr}_4$ ,  $\text{Cl}_4$ ,  $\text{CHI}_3$ ,  $\text{C}_2\text{Cl}_6$ ,  $\text{CBrCl}_3$ ,  $\text{CCl}_4$ ,  $\text{CHBr}_3$ ,  $\text{CHCl}_3$ ,  $\text{C}_2\text{Br}_6$ ,  $\text{C}_2\text{HBr}_5$ ,  $\text{C}_6\text{H}_5\text{CBr}_3$ ,  $\text{CIBr}_3$ ,  $\text{ClCl}_3$ ,  $\text{CHCl}_2$ ,  $\text{CHIBr}_2$ ,  $\text{CBrCl}_3$ ,  $\text{CHB}_2\text{Cl}_2$ ,  $\alpha$ ,  $\alpha$ ,  $\alpha$ -trichlorotoluene,  $\alpha$ ,  $\alpha$ ,  $\alpha$ -tribromoacetophenone and the like.

It is appropriate for further sensitization to carry out free radical sensitization in the presence of sensitizers as shown below.

Leuco base or carbinol base of triphenylmethane dye such as

leuco malachite green,

leuco crystal violet,

leuco methyl violet,

leuco opal blue, and

carbinol malachite green.

Styryl dye base such as 4-(4-dimethylaminophenyl-1,3-butadienyl) quinoline, 4-p-dimethylaminostyryl quinoline, 2-p-dimethylaminostyryl quinoline, 2-(4-dimethylaminophenyl-1,3-butadienyl) quinoline, and 10 2-p-dimethylstyrylbenzothiazole.

Cyanine dye base such as 2-[3-(1-ethyl-2-(1H)-quinolylidene)] propenyl quinoline, 2-[2-methyl-3-(3-ethyl-2(3H)-benzothiazolylidene) propenyl]benzothiazole, and 15 4-[(-ethyl-2(1H)-quinolylidene)methyl]quinoline.

Merocyanine dye base such as 3-ethyl-5-[[(3-ethyl-2(3H)-benzoxazolylidene) shodanine, 1-ethyl-3-[(3-ethyl-2(3H)-benzoxazolylidene]oxyindole, and 4-[(3-ethyl-2(3H)-benzoxazolylidene]-3-phenyl-5-(4H)-isooxazolone.

Secondary or tertiary arylamines such as diphenylamine, N-methylamine, N, N-dimethylaniline, N-ethylaniline, N, N-diethylaniline, phenyl- $\alpha$ -naphthylamine, phenyl- $\beta$ -naphthylamine, triphenylamine, and 25 N-methyldiphenylamine, N-benzylaniline.

Carbazoles such as carbazole, N-ethylcarbazole, N-methylcarbazole, N-phenylcarbazole, N-benzylcarbazole, N-vinylcarbazole, 3,6-dibromo-N-vinylcarbazole, and 3-chloro-N-ethylcarbazole.

Indoles such as indole, 2-methylindole, 1, 2-dimethylindole, 1-phenylindole, 4-chloroindole, and N-vinylindole.

Free radical sensitization may be carried out not only in liquid phase, but also in solid phase, for example, irradiating a solid photosensitive film.

The electrophotographic photosensitive material may be used for producing image by using various known means concerning charging and development such as corona discharge, magnet brush development, and electrophoresis development.

The following examples are given for illustrating the present invention, but by no means for restricting the present invention.

#### EXAMPLE 1

A sand-blasted aluminum plate was defatted with a mixture of ether and alcohol, coated with a liquid having the following formulation by a rotatory coater in such an amount that the dried coating film is 8 microns thick and dried by warm wind.

|    |                                                                                                                                                                                                        |        |
|----|--------------------------------------------------------------------------------------------------------------------------------------------------------------------------------------------------------|--------|
| 55 | Poly-9-vinylcarbazole<br>(Juvican M-170; trade<br>name, supplied by BASF)<br>(as control) or<br>cyanogenated poly-9-vinyl-<br>carbazole of nitrogen content<br>as shown in (1)-(5) of a table<br>below | 2.0 g. |
| 60 | Chlorobenzene                                                                                                                                                                                          | 40 ml. |
|    | Crystal Violet                                                                                                                                                                                         | 2.0 mg |

The resulting photosensitive plate was mounted on a rotatory electrometer to charge negatively and exposed to tungsten lamp. Irradiation time of period was measured at one-third decay and one-tenth decay of potential and reciprocal of the value of irradiation time of period was designated as "sensitivity". The "sensitivity"

ity" thus defined for various samples is listed in the table below. Initial potential when irradiation starts was about 500 volt for each sample.

5

| Cyanogenated poly-9-vinylcarbazole; nitrogen content | 1/3 decay | Sensitivity<br>1/10 decay |
|------------------------------------------------------|-----------|---------------------------|
| (1) 8.51 %                                           | 1.50      | 1.95                      |
| (2) 9.60 % (preparation Example 1)                   | 2.30      | 2.75                      |
| (3) 11.89 %                                          | 5.35      | 5.95                      |
| (4) 14.59 %                                          | 8.80      | 10.5                      |
| (5) 20.41 %                                          | 8.85      | 10.5                      |
| Poly-9-vinylcarbazole (control)                      | 1.0       | 1.0                       |

15

Cyanogenated poly-9-vinylcarbazole in (1) and (3) above were prepared by reacting an iodinated poly-9-vinylcarbazole with a sufficient amount of cuprous cyanide in a way similar to Preparation Example 1 and those in (4) and (5) above were prepared by reacting a brominated poly-9-vinylcarbazole with a sufficient amount of cuprous cyanide in a way similar to Preparation Example 3.

25

#### EXAMPLE 2

|                                                     |        |
|-----------------------------------------------------|--------|
| Polymer of No. 1 to No. 10 in Preparation Example 2 | 2.0 g. |
| Crystal Violet                                      | 5 mg.  |
| 2,4,7-Trinitrofluorenone                            | 2 mg.  |
| Diphenyl chloride                                   | 0.5 g. |
| Chlorobenzene                                       | 40 cc. |

30

The above formulation was applied to an art paper in an amount that the dried coating is 8 microns thick to produce a photosensitive paper. This was charged in a dark place and exposed to a light image formed by a photographic enlarger equipped with a 500 W tungsten lamp through a positive microfilm original. The resulting latent image was developed with liquid developer to give good positive images. Optimum exposure was 300 lux.second.

35

#### EXAMPLE 3

|                                                                    |         |
|--------------------------------------------------------------------|---------|
| Cyanogenated polymer as listed in (1) - (4) in a table shown below | 2.0 g.  |
| Carbon tetrabromide                                                | 100 mg. |
| 9-Vinylcarbazole                                                   | 180 mg. |
| Chlorobenzene                                                      | 40 cc.  |

45

A solution containing above ingredients was placed in an Erlenmyer flask of hard glass and was subjected to photochemical treatment with stirring for 5 minutes by a 100 W high pressure mercury lamp at a distance of 10 cm. Then, 2mg. of 2, 4, 7-trinitrofluorenone was added to the reaction liquid to form a photosensitive liquid. The resulting photosensitive liquid was coated on a high grade paper having a polyvinylalcohol layer on the surface to form a coating of 8 $\mu$  thick (after dried). The photosensitive paper thus obtained was corona-charged at a dark place and a light image was projected thereonto by using a photographic enlarger equipped with a 500 W tungsten lamp through a positive microfilm. The resulting electrostatic latent image was developed by using a liquid developer to form positive im-

50

55

ages. Exposure amount required for obtaining sharp and clear positive images is described as optimum exposure for cyanogenated polymers (1)-(4) in a table below.

| Cyanogenated polymers                                                                  | Nitrogen content (%) | Optimum exposure (lux. sec) |
|----------------------------------------------------------------------------------------|----------------------|-----------------------------|
| (1) Cyanogenated poly-9-vinyl carbazole                                                | 8.51                 | 150                         |
| (2) Cyanogenated poly-9-vinylcarbazole (obtained by Preparation Example 1)             | 9.60                 | 130                         |
| (3) Cyanogenated poly-9-vinyl carbazole                                                | 11.89                | 120                         |
| (4) Cyanogenated-chlorinated poly-9-vinylcarbazole (obtained by Preparation Example 4) | 8.36                 | 95                          |

Cyanogenated poly-9-vinylcarbazoles in (1) and (3) were prepared in a way similar to Preparation Example 1.

#### EXAMPLE 4

A sand-blasted aluminum plate was defatted with etheralcohol and coated with a liquid of the following composition by using a rotary coater to form a coating of 8 microns thick (after dried) and then dried with warm wind.

|                                                                                                                   |         |
|-------------------------------------------------------------------------------------------------------------------|---------|
| Poly-9-vinylcarbazole (Luvican M-170) (control) or photoconductive polymer produced by Preparation Example 7 or 8 | 2.0 g.  |
| Tetrahydrofuran                                                                                                   | 40 ml.  |
| 2,4,7-trinitrofluorenone                                                                                          | 1.0 mg. |

The resulting photosensitive plate was mounted on a rotary electrometer to charge negatively and exposed to tungsten lamp. Irradiation time of period was measured at one-third decay and one-tenth decay of potential, and reciprocal of the value of irradiation time period was designated as "sensitivity". The "sensitivity" thus defined for various samples is listed in the table below. Initial potential when irradiation starts was about 500 volt for each sample.

| Thiocyanated poly-9-vinylcarbazole, content of sulfur | 1/3 decay | Sensitivity<br>1/10 decay |
|-------------------------------------------------------|-----------|---------------------------|
| 3.85 %                                                | 2.2       | 2.6                       |
| 7.18 %                                                | 5.3       | 5.9                       |
| Poly-9-vinylcarbazole (control)                       | 1.0       | 1.0                       |

50

55

#### EXAMPLE 5

A photosensitive liquid was applied to a high grade paper (60 g/m<sup>2</sup>) having a polyvinylalcohol layer to form a coating of 8 microns thick (after dried) for producing a photosensitive paper.

The photosensitive liqued was prepared by dissolving 2 g. of cyanogenated 9-vinylcarbazole-ethyl acrylate copolymer or cyanogenated 9-vinylcarbazole-styrene copolymer as prepared in preparation Example 9 in 40 ml. of monochlorobenzene, adding 100 mg. of carbon tetrabromide and 2 mg. of triphenylbismuthine

13

thereto, irradiating with a 100 W high pressure mercury lamp at a distance of 10 cm. for 5 minutes to cause photochemical reaction, and then adding 5 mg. of 2, 4, 7-trinitrofluorenone thereto.

The resulting photosensitive paper was corona-charged in a dark place and exposed to a light image formed by a photographic enlarger equipped with a 500 W tungsten lamp through a positive microfilm original. The electrostatic image thus formed were developed with a liquid developer to obtain positive images of high contrast. Optimum exposure was 155 lux.-second for the former cyanogenated copolymer and 110 lux.second for the latter cyanogenated copolymer. Optimum exposure for the corresponding copolymer not cyanogenated was 465 lux.second and 310 lux.-second, respectively.

## EXAMPLE 6

|                      |         |
|----------------------|---------|
| Thiocyanated polymer | 2 g.    |
| Carbon tetrabromide  | 100 mg. |
| 9-Vinylcarbazole     | 50 mg.  |
| Triphenylbismuthine  | 2 mg.   |
| Monochlorobenzene    | 40 ml.  |

A solution composed of the above ingredients was subjected to photochemical reaction under the same conditions as in Example 5 and then 2 mg. of crystal violet was added thereto, and a photosensitive paper was prepared in a way similar to Example 5.

The resulting photosensitive paper was tested for image formation in a way similar to Example 5. The result is shown below.

| Thiocyanated polymer                                      | Optimum exposure |
|-----------------------------------------------------------|------------------|
| Thiocyanated poly-9-vinylcarbazole; sulfur content 3.85 % | 105 lux.second   |
| Thiocyanated copolymer produced by Preparation Example 3  | 160 lux.second   |
| Thiocyanated polymer produced by Preparation Example 4    | 90 lux.second    |

Polymers which sulfur content is low, for example, sulfure content is 3.85 %, gave satisfactory result even when triphenylbismuthine was removed from the above formulation.

We claim:

14

1. Electrophotographic photosensitive material which consists essentially of a polymer selected from the group consisting of (1) homopolymers of a thiocyanato-substituted 9-vinylcarbazole unit represented by the formula:



and (2) copolymers of said thiocyanato-substituted 9-vinylcarbazole with at least one monomer copolymerizable therewith.

2. The electrophotographic photosensitive material of claim 1 wherein said polymer is said copolymer (2) and said monomer is selected from the group consisting of an acrylic acid ester, a methacrylic acid ester and styrene.

3. Electrophotographic photosensitive material which consists essentially of a polymer selected from the group consisting of (1) homopolymers of a thiocyanato-substituted 9-vinylcarbazole unit represented by the formula:



40 wherein R is H, Cl, Br or I and wherein said homopolymer contains both monomer units where R is H and monomer units where R is Cl, Br or I; and (2) copolymers of said thiocyanato-substituted 9-vinylcarbazole with at least one monomer copolymerizable therewith.

45 4. The electrophotographic photosensitive material of claim 3 wherein said polymer is said copolymer (2) and said monomer is selected from the group consisting of an acrylic acid ester, a methacrylic acid ester and styrene.

\* \* \* \* \*

55

60

65

UNITED STATES PATENT OFFICE  
CERTIFICATE OF CORRECTION

Patent No. 3,917,482 Dated November 4, 1975

Inventor(s) TAKESHI EIDA, ET AL Page 1 of 2

It is certified that error appears in the above-identified patent and that said Letters Patent are hereby corrected as shown below:

On the cover page, between item [54] and [73] on the left hand column:

[75] Inventors: TAKESHI FIDA" should read --TAKESHI EIDA--

On the cover page, at [57] Abstract, the word "potosensitive" should read --photosensitive--

Column 2, line 47, "smoothyl" should read --smoothly--

Columns 3 and 4, in the Table, and Columns 5 and 6, in the Table, "Cyanate" should read --Cyanated--.

Column 5 and 6 in the Table, under the heading CN content #2, "0.374" should read --0.574--

In the Table at the bottom of Column 3 and 4, under the heading "chlorobenzene", third and last lines, insert --  $\Delta$  --.

In the Table at the top of Columns 5 and 6, under the heading "chlorobenzene", first line and under the heading "Solubility tetrahydrofuran", last line, insert --  $\Delta$  --.

Column 5, line 14, "soluble" should read --  $\Delta$  :soluble--

Column 7, line 55, "thereto" should read --thereto--

UNITED STATES PATENT OFFICE  
CERTIFICATE OF CORRECTION

Patent No. 3,917,482 Dated November 4, 1975

Inventor(s) TAKESHI EIDA, ET AL Page 2 of 2

It is certified that error appears in the above-identified patent and that said Letters Patent are hereby corrected as shown below:

Column 9, line 16, "oxtruded" should read --extruded--

Column 10, line 1, "grren" should read --green--

Column 10, line 12, delete "]" immediately after quinolylidene).

Column 10, line 49 and 64, "ratory" should read --rotary--

Column 12, line 63, "liquied" should read --liquid--

Column 13, line 47, "sulfure" should read --sulfur--

Column 10, line 12, insert --]- immediately after "propenyl".

Signed and Sealed this

thirteenth Day of April 1976

[SEAL]

Attest:

RUTH C. MASON  
*Attesting Officer*

C. MARSHALL DANN  
*Commissioner of Patents and Trademarks*